

H. J. YOUNG,  
FIBER PROCESS,  
APPLICATION FILED MAY 5, 1913.

1,146,987.

Patented July 20, 1915.

2 SHEETS—SHEET 1.



Witnesses

C. B. Foster

Oliver B. Kaiser

Homer J. Young

By Wood Wood & Nathan

Attorneys

H. J. YOUNG.  
FIBER PROCESS.  
APPLICATION FILED MAY 5, 1913.

1,146,987.

Patented July 20, 1915.

2 SHEETS—SHEET 2.



## Witnesses

C. B. Foster.

Oliver B. Kaiser

Homer J. Young

By Wm. Wm. & Nathan

Attorneys

# UNITED STATES PATENT OFFICE.

HOMER J. YOUNG, OF CINCINNATI, OHIO.

## FIBER PROCESS.

1,146,987.

Specification of Letters Patent. Patented July 20, 1915.

Application filed May 5, 1913. Serial No. 765,674.

*To all whom it may concern:*

Be it known that I, HOMER J. YOUNG, a citizen of the United States, residing at Cincinnati, in the county of Hamilton and State of Ohio, have invented certain new and useful Improvements in Fiber Processes, of which the following is a specification.

This invention deals with the liberation of hemp fiber from the plant, and it consists in a system embodying unique structures, characteristic relations, and treatments novel in nature and sequence whereby an essentially superior fiber may be derived from the stalk by a continuous operation and within a short time from its reception from the field, without rendering long time customary preliminary steps necessary.

The primary object of this invention is to devise a structural organization intimately and harmoniously related to a sequence of manipulative steps constituting an essentially commercial process, making for an inexpensive compact and self-contained manufacturing installation well adapted for an economic and rapid handling of hemp by starting with its natural condition as it is obtained from the field and culminating in skeins of fiber.

Other objects and advantages will be in part outlined in the following description and in part rendered apparent from the annexed drawings in connection therewith.

To enable others skilled in the art so fully to comprehend the underlying features thereof that they may embody the same by the numerous modifications in structure, relation, steps and sequence thereof contemplated by this invention, drawings depicting a preferred installation have been annexed as a part of this disclosure and in such drawings, like characters of reference denote corresponding parts throughout all the views, of which:

Figure 1 portrays in perspective one end of a building embodying my installation, showing the means instrumental in subjecting the hemp plants to certain initial steps of my process. Fig. 2 is a section taken through line 2—2 of Fig. 1, showing the construction of the retting tank. Fig. 3 is the same view of the rear end of the said building showing more clearly the final steps in the process resulting in a product bundled for commercial purposes. Fig. 4 is a detailed section taken in a vertical plane through line 4—4 of Fig. 1, showing more

clearly certain details of the plant elevator and the by-product classifier.

Continuing now by way of a more detailed description, it will be convenient to describe details of structure in connection with the disclosure of the steps of my process in the sequence in which they will preferably follow in practice.

It may be preliminarily stated that this installation may be conveniently made in connection with a two-storied building, utilizing the upper floor for preliminary operations and the lower floor for immediate delivery of raw material, as well as the concluding operations yielding the same as a finished product.

*Conveying plants to stalking machine.*—This operation is carried out in any appropriate way, depending upon the conditions of installation. Thus, in the preferred form the raw material is received on the ground floor and an elevator A delivers it to a concave receiving table on the upper floor. This elevator provides a table 1, upon which the attendant will place the material preparatory to pushing it through the opening 3 into a position determined by the comb 2, such that it may be effectively seized and conveyed upwardly by means of an endless belt 4 having rake-like prongs 5 and passing around appropriate pulleys within the elevator box. During their transit the plants will be dried by means of the steam pipes 7, which insure an elimination of any undue dampness in the plants, either initially had or acquired during their storage. By regulating the speed of the conveyer belt and adjusting the flow of steam in the pipes 7, the plants may be automatically correctly conditioned preparatory to the next following plowing, threshing and stripping operations.

That is to say, the leaf on the stalk, as well as the seed-pod, will be made crisp and dry. The stalk itself should also be well dried so that it will be split full length when subsequently run between the crushing rolls.

The dried plants are received upon the comb 6 of the concave table B, from which they are manually removed by an attendant stationed at this point, who feeds them into the stalking apparatus.

*Threshing, plowing and stripping the plants.*—This is done by means of a stalking machine C, which is intended to deliver the cleaned stalks, from which the fiber is subsequently obtained. The operator lays

the plants (butt-end to the left) on a steam table 8, and then feeds them laterally onto the traveling belt 9, so that they pass under the companion endless belt 10 and are thereby moved laterally to cause their blossom ends to pass under the action of the angularly positioned rollers 11, 12. It is to be noted that the table 8 has a lateral extension 13 upon which the leaf or flowering end rests while acted upon by the rollers 11 and 12. The one roller is a flayer, and thresher, *i. e.*, it has short lengths of straps, ropes or whips to break the seed-pods and thresh out the seeds, and the other roller is made of fiber wire or ratan, like a rotary brush, and it strips the leaf from the stalk and sweeps the leaf, the seeds and the pods all into a chute D that carries them downwardly to the lower floor to a classifier M, which will subsequently be explained. It is to be noted that while the plant passes through the elevator in the form of bundles, the attendant unbundles the plants at the table B, so that they pass through the stalking machine C and are finally delivered as separate stalks onto the table 14.

*Breaking stalks along fiber.*—The purpose of this operation is to break or crush the stalks so that the lines of cleavage will 30 run longitudinally, and open up the interior of the same to the action of the degumming solution and expedite that operation, and permit it to be performed with the least injury to the fibers. The table 14 may embody 35 a plurality of surface rollers acting automatically to propel the stalks toward the rollers 15 of the breaking machine E, it being noted that the stalks pass through such rollers butt-ends first, and from there onto 40 the table 16, the butt-ends being urged against the foot board 18 by the action of the surface rolls 17, so as to bring the stalks again into alignment suitable for their subsequent progression in a lateral direction 45 through the remaining steps. The rolls 15 are effective to crush all the large stalks without injury to the fiber by splitting them throughout their entire length, generally into quadrants. Rolls corrugated to break 50 the stalks somewhat are desirable also.

*Chemically retting the stalks.*—This operation is carried out automatically in a retting tank F. The attendant shifts the stalks from the foot-board 18 onto the portion 55 19 of the table, then pushes them laterally on to runners 20. An endless belt 21 carrying rake-teeth 22 passes around rolls or sprockets 23, 24 and 25, the two former being partially submerged and the latter being elevated as shown, so that the teeth engage 60 the stalks and carry them downwardly along the runners 20, which curve downwardly, as indicated by 29, passes through the tank 26 within a distance from the bottom 65 thereof, so that the stalks are carried

along while completely submerged in the tank solution until ultimately they are forced up the elevated end of the runners and onto the discharge board 30. Rods 30' assist in draining the saturated stock.

The tank is about 35 ft. long and it contains about a 2% caustic aqueous solution, and it is kept at about 200° F. For the purpose of more economically maintaining the temperature and carrying off fumes, the tank may be covered by the hood 27 leading to the discharge pipe 28. The stalk travels under solution for about 30 ft. and the conveyor travels the length of the tank in about fifteen minutes, and ordinarily about thirty 70 pounds of the dry stalk is fed per minute through the tank; the stalk being kept straight and separated in the form of small batches by the rows of teeth 22 on the belt. Of course, these figures are subject to modification in accordance with local considerations, but under the conditions named, this operation will suffice to effectively soften the gum or material cementing the fibers together, especially by reason of the preliminary longitudinal crushing of the stalks, whereby the solution gains access quickly to all portions thereof. The use of borax is also proposed.

*Washing and draining the stalks.*—This 95 operation is effected automatically by means of the apparatus G. The stalks are received from the board 30 onto the belt 31, which travels around guide rollers 32, 33, running considerably faster than the belt 21 so as to 100 spread the stalks apart and expose them thoroughly to the action of a washing and drenching spray. It is to be noted that these belts overlie a tank 34 which carries a neutralizing solution (about 1% acetic acid) which is pumped up by the pump 35 into the pipe 36 and then into the spray pipes 37, and out on the stalks and then back to the tank. This solution is preferably cold, and after the stalks have been 105 well rinsed and neutralized thereby they are received upon the comb 38 and directed transversely between the rotating rolls 39 and 40, which act as a squeegee, and squeeze out about 40% more or less of the fluid. 110 The efficiency of this squeegee is enhanced by reason of the fact that the stalk fed therethrough is first broken.

*Drying and softening the stalks.*—This is done in the evaporator H, into which the 115 stalks are carried by the endless belt 41 that passes around rolls 42 and 43, and through a closed chamber 44, preferably having an outlet vent 45 to take off vapors. By means of an inlet pipe 46 and suitable steam pipes 47, the interior of the evaporator H is maintained as nearly at a uniform temperature as possible, which temperature is preferably at about 200° F. and the speed of the belt 41 is such that it is subjected to a forced evap- 130

oration for about twenty-five minutes. Inasmuch as the stalk has first been crushed or broken, as before stated, the drying by this evaporator is greatly expedited since the 5 stalks are exposed both within and without to the immediate effects of the temperature.

Although the stalk has been evaporated in the presence of steam, it has a tendency to harden unduly and dry superficially and 10 somewhat strengthen the fiber cementing material and the outer husk, and to counter this I propose to spray or atomize hemp-seed oil obtained from the pipe 48 and delivered by the spray pipes 49. This will be quickly 15 absorbed by the fiber tending to toughen and render it more pliable, but without disadvantageously affecting the whole or body of the stalk from the standpoint of the ultimate breaking operation. This oiling step 20 conditions the fiber and helps make it suitable for use by the spinners. The fibers will contain not more than 4% of the oil.

*Tippling the stalks.*—When the stalks reach the end of the belt 41 they are received on one or the other side of the tipple I, which consists of a member having stalk-receiving arms 51, and eccentrically pivoted at 52 so that whenever a predetermined weight of stalk accumulates it will automatically tilt and throw the material to one side or the other into chutes 53 and 54 as the case may be. This tipple in this way determines the proper amount for each skein or fiber which will be ultimately produced.

35 *End-alining the stalks before breaking.*—This is accomplished by means of the chutes J, which have slides 55, 56 extending at an angle of about 45° from the hoppers 53, 54. The butt-ends of the stalks are brought 40 against suitable gates preparatory to entering the breaking rolls, and are thereby brought into alinement, so that the fibers in the skeins will be similarly alined.

45 *Isolating the fibers from the hulls.*—This is accomplished by means of hemp brakes K wherein the stalks are spread and automatically fed between crimping rolls that partially mesh, so as to break the hulls of the stalk transversely into small pieces less than 50 an inch long, so that the rolls will have differential movements, causing the fiber to pucker and forcing out the broken hulls. Such hulls are drawn away by means of throw pipes 57 into the loft above and may 55 be utilized as a by-product for paper pulp and other purposes.

60 *Skeining the fibers.*—This is facilitated by means of "horses" indicated by L, preferably in pairs, and in the form of elongated narrow tables; the fore part of which provides a closed top 58 about four feet long, across which the operator may throw the skeins as fast as they are received from the hemp-brakes, and facilitates tying the middle of the skeins by means of a piece of tow

or short-length fiber. The tied skein is then advanced by hand until one of the teeth of the endless belt 59 engages its middle and conveys it to the baler, and it is noteworthy that two "horses" act in conjunction with 70 the baler between their terminals, so that the skeins or hanks may be packed in conversely arranged layers, alternately lying in opposite directions.

75 *By-product classifier.*—Reverting to the stripping, threshing and flaying mechanism C, it will be recalled that the leaf, seeds, pods and stems removed from the stalks will pass down the chute of the classifier D and will drop through a side blast of air 80 (issuing through screen 62 from pipe 61) so that the lighter particles of leaf will be blown into passage 63 and drop into the leaf receptacle 64. The heavier seeds, etc., will fall down passage 65 onto a shaking screen 85 66, through which the seeds will pass (together with some dirt) and thence onto screen 67 (dirt goes through into the box 69) and the seeds then pass into box 68, from which they are removed and oil extracted therefrom, or otherwise disposed of. The pods, etc., will pass down into box 70.

90 Without further elaboration, the foregoing will so fully reveal the gist of this invention that others can by applying current 95 knowledge readily adapt it for various applications without omitting certain features that, from the standpoint of the prior art, fairly constitute essential characteristics of the generic or specific aspects of this invention, and therefore such adaptation should and is intended to be comprehended within the meaning and range of equivalency of the following claims.

100 Having thus revealed this invention I 105 therefore claim as new and desire to secure by Letters Patent of the United States:—

1. A process of liberating hemp-fiber, consisting in isolating the stalks from the plant structure, then passing said stalks lengthwise between rollers to break the same in longitudinal planes, then submerging said broken stalks in a heated solution adapted to soften the fiber cementing material, then removing said stalks and mechanically 110 eliminating excess solution therefrom, then reducing the contained moisture in said stalks by passing the same through a heated evaporating oven, then spraying the sufficiently dried stalks with oil, and then transversely breaking said stalks and eliminating the fiber therefrom.

115 2. A process of liberating hemp-fiber, consisting in isolating the stalks from the plant structure, then passing said stalks lengthwise between rollers to break the same in longitudinal planes, then submerging said broken stalks in a heated solution adapted to soften the fiber cementing material, then removing said stalks and mechanically 120 125 130

eliminating excess solution therefrom, then reducing the contained moisture in said stalks by passing the same through a heated evaporating oven, and then transversely 5 breaking said stalks and eliminating the fiber therefrom.

3. A process of liberating hemp-fiber, consisting in first isolating the stalk from the plant, then passing the stalks endwise between crushing rollers to break the same longitudinally and internally open said stalks to the entry of solvent, then submerging said stalks for a short period in a 10 2% solution of alkali at 200° F., then drying said stalks, then mechanically liberating the fiber therefrom.

4. A process of liberating hemp-fiber, consisting in first isolating the stalk from the plant, then passing the stalks endwise between crushing rollers to break the same longitudinally and internally open said stalks to the entry of solvent, then submerging said stalks for a short period in a 2% 20 solution of alkali at 200° F., then removing said stalks and rinsing the same with an acidulated solution, then eliminating excess moisture from said stalks, and then mechanically liberating the fiber therefrom.

5. A process of liberating hemp-fiber, consisting in first isolating the stalk from the plant, then passing the stalks endwise between crushing rollers to break the same 30

longitudinally and internally open said stalks to the entry of solvent, then submerging said stalks for a short period in a 2% 35 solution of alkali at 200° F., then removing said stalks and rinsing the same with an acidulated solution, then passing said stalks through a squeegee to drain the same, then reducing the moisture content by a forced 40 evaporation and finally mechanically liberating the fiber from said stalks.

6. A process of liberating hemp-fiber, consisting in isolating the stalk from the plant, then conveying said stalks through a solution at about 200° F., for a short period, then rinsing said stalks in acidulated solution and mechanically separate excess solution therefrom, then drying the same by a forced evaporation, then treating said stalks 45 with a softening material and finally liberating the fiber therefrom.

7. A process of liberating hemp-fiber, consisting in softening the fiber cement material of the fibers of the stalk, then atomizing 55 hemp-seed oil under same to soften said stalks, and then mechanically liberating the fiber of said stalk.

In testimony whereof, I have hereunto set my hand.

HOMER J. YOUNG.

Witnesses:

ALBERT F. NATHAN,  
LOUISE A. BECK.